# EUROPEAN PATENT APPLICATION

(11) **EP 1 394 241 A1**
(43) Date of publication of application: **03.03.2004**
(21) Application number: 03254689.7
(22) Date of filing: 28.07.2003
(51) Int. Cl.: C10M 135/16

(54) **Cyclic thioureas as additives for lubricating oils**

(30) Priority: 07.08.2002 US 401540 P
(71) Applicant: ROHM AND HAAS COMPANY, Philadelphia, Pennsylvania 19106-2399 (US)
(72) Inventor: Mukkamala, Ravindranath, Lansdale, Pennsylvania 19446 (US)
(74) Representative: Kent, Venetia Katherine

(57) **Abstract**

A composition comprising: (a) from 0.1% to 20% of at least one cyclic thiourea compound of formula I: wherein W is O or S; R¹ and R² independently are hydrogen, alkyl, alkenyl, aryl or aralkyl; R³ and R⁴ independently are hydrogen, alkyl, alkenyl, aryl or aralkyl, or R³ and R⁴ groups combine with ring carbon atoms to which they are attached to form a five- to seven-membered heterocyclic ring; and (b) a lubricating oil.

## Description

### Background

This invention relates generally to cyclic thioureas useful as additives for lubricating oils.

Zinc dialkyldithiophosphates (ZDDP) are widely used as lubricant additives. The principal disadvantages of these compounds are that an ash residue is produced by the zinc as the additive is consumed, and that phosphorus is known to affect the efficiency of catalytic converters in motor vehicles, thereby causing emissions problems. Cyclic thiourea compounds useful as lubricant additives are disclosed in U.S. Patent No. 5,935,913. However, the compounds disclosed therein are not within the scope of the present invention.

The problem addressed by this invention is to find additional non-metallic, non-phosphorus-containing oil-soluble additives for lubricating oils.

### Statement of Invention

The present invention is directed to a composition comprising:
(a) from 0.1% to 20% of at least one cyclic thiourea compound of formula I: wherein W is O or S; R¹ and R² independently are hydrogen, alkyl, alkenyl, aryl or aralkyl; R³ and R⁴ independently are hydrogen, alkyl, alkenyl, aryl or aralkyl, or R³ and R⁴ groups combine with ring carbon atoms to which they are attached to form a five- to seven-membered heterocyclic ring; and
(b) a lubricating oil.

The present invention is further directed to a method for improving the anti-wear characteristics of a lubricating oil by adding from 0.1% to 20% of a compound of formula I.

### Detailed Description

All percentages are weight percentages based on the entire composition described, unless specified otherwise. An "alkyl" group is a saturated hydrocarbyl group having from one to twenty-two carbon atoms in a linear, branched or cyclic arrangement, and having from 0 to 2 oxygen, nitrogen or sulfur atoms. Substitution on alkyl groups of one or more halo, hydroxy, alkoxy, alkanoyl or amido groups is permitted; alkoxy, alkanoyl and amido groups may in turn be substituted by one or more halo substituents. In one preferred embodiment, alkyl groups contain from one to twelve carbon atoms and from 0 to 1 oxygen, nitrogen or sulfur atoms; in another preferred embodiment, alkyl groups contain from 12 to 22 carbon atoms, and more preferably, no heteroatoms. An "alkenyl" group is an "alkyl" group in which at least one single bond has been replaced with a double bond. An "aryl" group is a substituent derived from an aromatic compound, including heterocyclic aromatic compounds having heteroatoms chosen from among nitrogen, oxygen and sulfur. An aryl group has a total of from five to twenty ring atoms, and has one or more rings which are separate or fused. Substitution on aryl groups of one or more halo, alkyl, alkenyl, hydroxy, alkoxy, alkanoyl or amido groups is permitted, with substitution by one or more halo groups being possible on alkyl, alkenyl, alkoxy, alkanoyl or amido groups. An "aralkyl" group is an "alkyl" group substituted by an "aryl" group. A "lubricating oil" is a natural or synthetic oil, or a mixture thereof, having suitable viscosity for use as a lubricant, e.g., as crankcase oil in an internal combustion engine, automatic transmission fluid, turbine lubricant, gear lubricant, compressor lubricant, metal-working lubricant, hydraulic fluid, etc.

In one embodiment of the invention, preferably formula (I) has R¹, R², R³ and R⁴ which independently are hydrogen, alkyl, alkenyl, aryl or aralkyl, i.e., the compound is not bicyclic. Preferably, R¹, R², R³ and R⁴ independently are hydrogen, alkyl or alkenyl, more preferably at least one of R¹, R², R³ and R⁴ is C₆-C₂₂ alkyl or alkenyl, more preferably at least one of R¹, R², R³ and R⁴ is C₁₀-C₂₂ alkyl, and most preferably at least one of R¹, R², R³ and R⁴ is C₁₆-C₂₂ alkyl.

In another embodiment of the invention R³ and R⁴ groups in formula I combine with ring carbon atoms to which they are attached to form a five- to seven-membered heterocyclic ring. In a preferred embodiment R³ and R⁴ groups combine to form the following bicyclic system of formula (II): wherein R⁵ and R⁶ independently are hydrogen, alkyl, alkenyl, aryl or aralkyl. In a preferred embodiment of the invention, in which W is O, R¹ and R⁶ are the same, and R² and R⁵ are the same, the compound is a symmetric bicyclic compound of formula (III):

In one embodiment of the invention, a compound of formula (I) is prepared from a 2-amino alkyl nitrile and carbon disulfide, as shown below: Preferably, R² is C₆-C₂₂ alkyl or alkenyl, more preferably C₁₀-C₂₂ alkyl, and most preferably C₁₆-C₂₂ alkyl. Preferably, R² is derived from an unsubstituted C₁₆-C₂₂ alkyl amine, R²NH₂, preferably one which is an oil-soluble amine. In one preferred embodiment, the alkyl amine is a tertiary alkyl primary amine., i.e., a primary amine in which the alkyl group is attached to the amino group through a tertiary carbon. Examples of commercially available tertiary alkyl primary amines are the Primene^{TM} amines available from Rohm and Haas Company, Philadelphia, PA.

In one embodiment of the invention, a compound of formula (III) is prepared from a substituted thiourea and a di-ester of acetylenedicarboxylic acid, as shown below: The R groups are alkyl, alkenyl, or aralkyl groups, preferably C₁-C₄ alkyl groups. Preferably, R¹ and R² are hydrogen, alkyl or alkenyl, more preferably at least one of R¹ and R² is C₆-C₂₂ alkyl or alkenyl, more preferably at least one of R¹ and R² is C₁₀-C₂₂ alkyl, and most preferably at least one of R¹ and R² is C₁₆-C₂₂ alkyl.

In one embodiment of the invention, a compound of formula (I) is prepared from a substituted thiourea and an ester of a α,β-unsaturated carboxylic acid, as shown below: Preferably, R³ and R⁴ are hydrogen or C₁-C₄ alkyl. Preferably, R¹ and R² are hydrogen, alkyl or alkenyl, more preferably at least one of R¹ and R² is C₆-C₂₂ alkyl or alkenyl, more preferably at least one of R¹ and R² is C₁₀-C₂₂ alkyl, and most preferably at least one of R¹ and R² is C₁₆-C₂₂ alkyl.

Preferably, the compound(s) of formula (I) is present in a lubricating oil in a total amount of at least 0.2%, more preferably at least 0.3%, and most preferably at least 0.4%. Preferably, the compound(s) of formula (I) is present in a lubricating oil in a total amount no greater than 10%, more preferably no greater than 5%, and most preferably no greater than 2%. Preferably, the compounds are soluble at the aforementioned levels.

Optionally, other additives typically used in lubricating oils are present in the composition. Such additives include, but are not limited to, other anti-wear additives, anti-corrosion additives, dispersants, detergents, antioxidants, antifoamants, friction modifiers, seal swell agents, demulsifiers, viscosity index improvers and pour point depressants. Other anti-wear additives that can be used in combination with the compound of formula (I) include the commercial products known as ZDDP, which are zinc dialkyldithiophosphates. In addition to improving the anti-wear characteristics of lubricating oils, the compound of formula (I) typically also improves anti-corrosion characteristics and functions as an anti-oxidant.

## Claims

1. A composition comprising:
(a) from 0.1% to 20% of at least one cyclic thiourea compound of formula I: wherein W is O or S; R¹ and R² independently are hydrogen, alkyl, alkenyl, aryl or aralkyl; R³ and R⁴ independently are hydrogen, alkyl, alkenyl, aryl or aralkyl, or R³ and R⁴ groups combine with ring carbon atoms to which they are attached to form a five- to seven-membered heterocyclic ring; and
(b) a lubricating oil.

2. The composition of claim 1 in which W is O, and R¹, R², R³ and R⁴ independently are hydrogen, alkyl, alkenyl, aryl or aralkyl.

3. The composition of claim 2 in which R¹, R², R³ and R⁴ independently are hydrogen or alkyl.

4. The composition of claim 3 in which at least one of R¹, R², R³ and R⁴ is C₆-C₂₂ alkyl.

5. The composition of claim 1 in which W is S, and R¹, R², R³ and R⁴ independently are hydrogen, alkyl, alkenyl, aryl or aralkyl.

6. The composition of claim 1 in which R³ and R⁴ groups combine with ring carbon atoms to which they are attached to form a five- to seven-membered heterocyclic ring.

7. The composition of claim 6 in which the cyclic thiourea has formula wherein R⁵ and R⁶ independently are hydrogen, alkyl, alkenyl, aryl or aralkyl.

8. The composition of claim 7 in which W is O, R¹ and R⁶ are the same, and R² and R⁵ are the same.

9. The composition of claim 8 in which R¹ and R² independently are hydrogen or alkyl.

10. The composition of claim 9 in which at least one of R¹ and R² is C₆-C₂₂ alkyl.
